# EUROPEAN PATENT SPECIFICATION

(11) **EP 0 265 402 B1**
(45) Date of publication and mention of the grant of the patent: **28.08.1991**
(21) Application number: 87850292.1
(22) Date of filing: 28.09.1987
(51) Int. Cl.: C22C 38/60, C22C 38/00

(54) **Calcium treated boron alloyed steel with improved machinability**
Mit Kalzium behandelter, Bor enthaltender Stahl mit verbesserter Zerspannbarkeit
Acier traité au calcium et contenant du bore, présentant une meilleure usinabilité

(30) Priority: 29.09.1986 FI 863918
(43) Date of publication of application: 27.04.1988
(73) Proprietor: Ovako Steel Oy AB, 00100 Helsinki (FI)
(72) Inventor: Ollilainen, Vesa, SF-55610 Imatra (FI); Pöntinen, Hannu, SF-55610 Imatra (FI); Paju, Martti, SF-55800 Imatra (FI)
(74) Representative: Wibom, Hans Sven Erik

(56) References cited:
- FR-A- 2 088 862
- US-A- 2 388 214
- US-A- 3 634 073
- US-A- 4 265 660

## Description

The object of the present invention is improved machinable calcium treated boron alloyed steel, wherein a free boron content sufficient for hardenability is obtained without Ti and/or Al contents disadvantageous to machinability. With this invention the weaknesses of the known techniques are avoided.

In the known heat treated boron alloyed steels the free boron content sufficient for hardenability is obtained by binding the dissolved nitrogen aluminium and/or titanium. The machinability of the known steels is poor for the following reasons:
- As a result of titanium alloying (about 0.02-0.05 wt-%) required to protect boron, the steel contains extremely hard large TiN particles which have a disadvantageous effect on machinability.
- The high Al content (0.05-0.1 wt-%) required to protect the boron impairs machinability.
- The machinability of boron steels of these known types cannot be essentially improved by calcium treatment.

A summary of the invention is presented in the following.

In the steel of the present invention amounts of Al and Ti added are so low that they do not bind all the dissolved nitrogen. The excessive part of nitrogen, which remains after the binding by titanium and aluminium, is bound to boron to give boron nitrides. A sufficient amount of boron is alloyed so that in addition to the boron in nitrides, the steel contains about 10-30 weight-ppm chemically free boron.

Titanium alloying is restricted to prevent the precipitation of large so-called primary titanium nitrides in the molten state. The maximum amount of titanium added depends on the nitrogen content of the steel. If desired, the titanium may be left out altogether. At least 0.005 wt-% of aluminium is alloyed in order to kill the steel, to reduce the grain size and to obtain the correct type of non metallic inclusions. Aluminium contents of over 0.014 wt-% are not alloyed due to the deterioration of machinability.

It is also characteristic for the steel of the present invention that it has been calcium treated in ladle. The calcium treatment improves the machinability of the steel. Full advantage is gained from the calcium treatment because high Ti or Al contents are not used.

It is furthermore characteristic for the steel of the present invention that it contains the following alloying elements shown below in percentages by weight:
carbon 0.01 - 0.50%
silicon 0.01 - 2.00%
manganese 0.40 - 1.60%
sulphur 0.01 - 0.30%
chromium 0 - 2.00%
molybdenum 0 - 0.80%

The use of the steel determines the alloying element combination selected.

The steel of the present invention is given in claim 1.

In the following the technological background of the invention and the test results obtained with the steels relating to the invention will be described.

Boron is an element which intensifies the hardenability of steel considerably with very low contents of chemically free boron.

It is characteristic for the hardenability intensifyig effect of boron that maximum effect is obtained with a certain free boron content (0.001-0.004 wt-%) and that the obtained increase in hardenability diminishes as the carbon and alloying element contents increase.

Since boron has a hardenability intensifying effect only when it is dissolved in steel in chemically free form, it should be ensured that boron is not bound in compounds - mainly BN or B₂O₃ - or that the free boron content is the said 0.001-0.004 wt-% also after a part of the boron is bound in the above-mentioned compounds.

In the established steel making technique, the obtaining of a stable hardenability effect of boron is ensured by adding nitrogen binding elements such as Ti and/or Al (also Zr, V, Nb) and a standard amount of boron after a thorough deoxidation.

It is also possible to alloy so much boron that although a part of it is bound in BN, enough boron still remains to guarantee the hardenability effect. This requires, however, advanced steel making technique because insufficiently low boron alloying results in the loss of hardenability and excessively high alloying in a decrease in hardenability and furthermore makes the steel brittle.

The increase in hardenability achieved by boron alloying, that is, the boron hardenability effect (Bf) is usually defined as the ratio of the ideal critical diameter (DI) measured by the Jominy-test (SFS-standard 2375) to the ideal critical diameter (DIchem) calculated on the basis of the chemical analysis (excluding boron):
Bf = DI/DIchem

The chemical analyses of the test steels are given in Table 1 and the results of their hardenability tests are shown in Table 2. The test results clearly show that the boron hardenability effect is achieved on exceeding a certain value of the ratio B/(N - Ti/3.4), wherein B is the boron content, N the nitrogen content and Ti the titanium content in percentages by weight. The intensity of the effect increases rapidly at first as the free boron content increases, but reaches then its maximum value which is dependent on the carbon and alloying element contents. The boron hardenability effect is thus achieved without Al and/or Ti alloying with a sufficiently high boron content.

The conventional boron-protecting methods, titanium and/or aluminium alloying, impair machinability. Titanium forms extremely hard cubic TiN particles which wear machining tools abrasively. This is shown by the shorter tool life when machining titanium alloyed steels. Fig. 1.

By means of calcium treatment the machinability of steel is improved by modifying non metallic inclusions. Oxides in untreated steels (aluminium oxides, silicates) are extremely hard and thus wear the machining tool abrasively. In calcium treated steels oxides are softer and in addition enveloped by a soft sulphide case. These modified non metallic inclusions cause less abrasive wear of machining tools. At high machining speeds the inclusions of calcium treated steel also form a protecting film on the surfaces of machining tools. Thus, the tool lives are substantially longer when machining calcium treated steels. Fig. 2.

The calcium treatment does not, however, affect the titanium nitride particles. Therefore, the machinability of titanium protected boron steel cannot be improved by calcium treatment. Fig. 3.

When aluminium is used to protect boron, the aluminium contents required are high which is known to impair the machinability of steel.

When the protection of boron is carried out according to the present application by means of excess boron alloying fixed to the nitrogen content of the steel, high titanium and/or aluminium contents are not required. The impairment of machinability caused by the above-mentioned alloying elements can thus be avoided,and an overall improvement of machinability is achieved by calcium treatment. Fig. 4.

Into the steel of the present invention it is also alloyed at least 0.01% sulphur because it is well known that sulphur addition improves machinability.

## Claims

1. Calcium treated hardenable boron alloyed steel, **characterized** in that the steel combines both an improved machinability and a hardenability intensifying effect of boron and the chemical composition of the steel in percentages by weight is:
carbon 0.01 - 0.5%
silicon 0.01 - 2.0%
manganese 0.4 - 1.6%
sulphur 0.01 - 0.3%
chromium 0 - 2.0%
molybdenum 0 - 0.8%
boron 0.002 - 0.02%
titanium 0 - 0 .015%
aluminium 0.005 - 0.014%
calcium 0.0015 - 0.01%
the balance being iron + impurities
and in addition wherein B is the boron content, N the nitrogen content and Ti the titanium content in percentages by weight.

2. Steel as claimed in claim 1, **characterized** in that the contents of boron and titanium in percentages by weight are:
boron 0.004 - 0.02%
titanium 0 - 0.005%.

3. Steel as claimed in claim 1, **characterized** in that the contents of boron and titanium in percentages by weight are:
boron 0.007 - 0.02%
titanium 0 - 0.005%.

4. Steel as claimed in claim 1, **characterized** in that the content of titanium in percentage by weight is 0.005 - 0.015%.

5. Steel as claimed in any one of the claims 1 - 4, **characterized** in that the content of sulphur in percentage by weight is 0.01 - 0.015%.

6. Steel as claimed in any one of the claims 1 - 4, **characterized** in that the content of sulphur in percentage by weight is 0.01 - 0.05%.

7. Steel as claimed in any one of the claims 1 - 6, **characterized** in that 0.1 - 1.5 kg of calcium is added per ton of molten steel with a lance.

8. Steel as claimed in claim 7, **characterized** in that the calcium is added as cored wire.

9. Steel as claimed in claim 7, **characterized** in that the calcium is added as capsules or briquettes.

## Revendications

1. Acier allié trempant au bore, traité au calcium, caractérisé en ce que cet acier jouit à la fois d'une aptitude améliorée à l'usinage et d'un effet, dû au bore, de renforcement de la trempabilité, et en ce que la composition chimique de l'acier, en pourcentages pondéraux, est la suivante : le complément étant constitué par le fer et des impuretés, et en ce qu'en plus où B représente la teneur en bore, N la teneur en azote et Ti la teneur en titane, en pourcentages pondéraux.

2. Acier conforme à la revendication 1, caractérisé en ce que les teneurs en bore et en titane sont les suivantes, en pourcentages pondéraux :

3. Acier conforme à la revendication 1, caractérisé en ce que les teneurs en bore et en titane sont les suivantes, en pourcentages pondéraux :

4. Acier conforme à la revendication 1, caractérisé en ce que la teneur en titane, en pourcentage pondéral, vaut de 0,005 à 0,015%.

5. Acier conforme à l'une quelconque des revendication 1 à 4, caractérisé en ce que la teneur en soufre, en pourcentage pondéral, vaut de 0,01 à 0,015%.

6. Acier conforme à l'une quelconque des revendications 1 à 4, caractérisé en ce que la teneur en soufre, en pourcentage pondéral, vaut de 0,01 à 0,05%.

7. Acier conforme à l'une quelconque des revendications 1 à 6, caractérisé en ce que l'on ajoute, avec une lance, de 0,1 à 1,5 kg de calcium par tonne d'acier fondu.

8. Acier conforme à la revendication 7, caractérisé en ce que le calcium est ajouté sous forme de fil à âme.

9. Acier conforme à la revendication 7, caractérisé en ce que le calcium est ajouté sous forme de capsules ou de briquettes.

## Patentansprüche

1. Kalziumbehandelter, härtbarer, borlegierter Stahl, der eine verbesserte Zerspanbarkeit und einen durch Bor hervorgerufenen, härtbarkeitssteigernden Effekt in sich vereint, dadurch gekennzeichnet, dass er die folgenden Legierungsbestandteile in den angegebenen gewichtsprozentualen Mengen enthält: und zusätzlich: wobei B den Borgehalt, N den Stickstoffgehalt und Ti den Titangehalt in Gewichtsprozent bedeuten.

2. Stahl gemäss Anspruch 1, dadurch gekennzeichnet, dass die gewichtsprozentualen Gehalte an Bor und Titan betragen:

3. Stahl gemäss Anspruch 1, dadurch gekennzeichnet, dass die gewichtsprozentualen Gehalte an Bor und Titan betragen:

4. Stahl gemäss Anspruch 1, dadurch gekennzeichnet, dass der gewichtsprozentuale Gehalt an Titan 0,005 - 0,015% beträgt.

5. Stahl gemäss einem der Ansprüche 1 bis 4, dadurch gekennzeichnet, dass der gewichtsprozentuale Gehalt an Schwefel 0,01 - 0,015% beträgt.

6. Stahl gemäss einem der Ansprüche 1 bis 4, dadurch gekennzeichnet, dass der gewichtsprozentuale Gehalt an Schwefel 0,01 - 0,05% beträgt.

7. Stahl gemäss einem der Ansprüche 1 bis 6, dadurch gekennzeichnet, dass pro Tonne Flüssigstahl 0,1 - 1,5 kg Kalzium mit einer Lanze zugegeben wird.

8. Stahl gemäss Anspruch 7, dadurch gekennzeichnet, dass das Kalzium als Seelendraht zugesetzt wird.

9. Stahl gemäss Anspruch 7, dadurch gekennzeichnet, dass das Kalzium in Form von Kapseln oder Briketts zugesetzt wird.
